

Dec. 31, 1968

J. F. HOULE ET AL

3,419,406

COATING COMPOSITIONS

Filed Aug. 4, 1967

FIG. 1



FIG. 2



JAMES F. HOULE  
GILDEN R. VAN NORMAN  
INVENTORS

*Walter O. Johnson*  
BY  
*W. H. Dowell*

ATTORNEY & AGENT

3,419,406  
COATING COMPOSITIONS

James F. Houle and Gilden R. VanNorman, Rochester, N.Y., assignors to Eastman Kodak Company, Rochester, N.Y., a corporation of New Jersey  
Continuation-in-part of application Ser. No. 347,931, Feb. 27, 1964, now Patent No. 3,342,601, dated Sept. 19, 1967. This application Aug. 4, 1967, Ser. No. 658,559

5 Claims. (Cl. 106—287)

## ABSTRACT OF THE DISCLOSURE

Aqueous solutions of complexes of titanium compounds render substrates hydrophilic, for example, a solution resulting from the addition of hydrogen peroxide, phosphoric acid and tetraisopropyl titanate to water when coated on an aluminum support renders the support hydrophilic.

This is a continuation-in-part application of U.S. Ser. No. 347,931 filed Feb. 27, 1964, by James F. Houle and Gilden R. VanNorman, now U.S. Patent 3,342,601.

This invention relates to lithographic printing plates, more particularly to offset printing plates commonly used in the lithographic trade.

Lithographic plates are well known in the graphic arts field, particularly those having metal supports such as aluminum or zinc. In recent years aluminum has been particularly attractive for lithographic plates due to its cost, availability and light weight. However, when aluminum is used as a substrate for printing plates, certain inherent disadvantages must first be overcome. For instances, it has been established that the naturally occurring oxide film on aluminum is not sufficiently hydrophilic to provide trouble-free operation on a lithographic printing press. The bare aluminum is prone to become slightly hydrophobic or oleophilic resulting in a gradual buildup of ink on the nonprinting areas. This phenomena is referred to in the trade as toning or scumming. In order to eliminate toning or scumming, a suitable, permanently hydrophilic surface which is relatively insoluble must be provided. Aluminum is also known to react with certain sensitive materials, such as diazo resins coated thereon, as indicated in U.S. Patent 2,714,066.

Several methods of imparting an insoluble, permanently hydrophilic surface to the aluminum substrate have been suggested in the prior art. Typical treatments include "anodizing," coating the surface with a hydrophilic organic polymer, etc. For instance, a method is described in French Patent 904,255, published Oct. 31, 1945, showing chemical or electrical treatments which provide a porous layer of aluminum compounds of oxygen, fluorine or phosphorous. In addition, Clerc, in the "Ilford Manual of Process Work," 1946, page 237, discloses treatment of aluminum plates with solutions containing fluosilicic acid or a fluosilicate.

These treatments, however, have not been satisfactory in producing a suitable hydrophilic coating on the aluminum adequate to provide the required ink-water differential for successful operation on a lithographic press. Moreover, the above treatments do not protect conventional diazo coatings from the aluminum so that the plates can be presensitized and stored over long periods of time prior to usage.

One method of providing an aluminum plate having an insoluble, hydrophilic layer which also isolates the diazo light sensitive coating from the aluminum substrate is to deposit a coating on the aluminum of a silicate containing the  $\text{SiO}_2$  radical.

A presensitized aluminum lithographic plate having a silicate layer thereon, has limited press life and also is subject to decreases in sensitivity during storage, especially after the plate has been exposed to the atmosphere particularly with high humidity or heat or a combination of both. Therefore, it has been desirable to provide a plate having greater press latitude, longer press life and longer shelf life than provided by the plates of the prior art.

Coating an aluminum surface with silica or similar silicate undercoating requires a smooth aluminum surface. However, it has customarily been found in lithographic printing that a grained or brushed surface provides a wider set of operating conditions on the press, particularly since a grained plate requires a less critical ink-water balance than does the silicate coated smooth plate. Moreover, the less critical ink-water balance decreases the tendency for the ink to emulsify during multicolor printing, which normally results in a loss of image sharpness. Therefore, it has also been desirable to provide a presensitized aluminum plate having a grained or brushed surface.

In order to provide an insoluble hydrophilic surface or surface coating it is desirable to eliminate the necessity of elevated temperatures and subsequent washing during the process. These steps are essential in many of the known processes. It is also desirable that the treatment be conducted from aqueous media thus eliminating toxic or flammable solvent vapors. Therefore, to achieve improved characteristics for a presensitized plate, it is desirable to obtain a plate having a grained surface, an improved method of treatment to provide a hydrophilic surface and a stabilized light sensitive coating thereon, thus giving a combination of superior printing and keeping qualities.

We have found that a suitable insoluble, hydrophilic surface layer may be imparted to an aluminum sheet by treatment with aqueous solutions of certain complex titanium salts capable of reacting at or on the surface to form an insoluble layer.

One object of this invention is to provide a hydrophilic lithographic printing surface. Another object is to provide a coating composition for treating surfaces such as metal, paper, polymeric, etc. to render a surface hydrophilic for use in lithographic printing. A further object is to provide a presensitized lithographic printing plate. A still further object is to provide a diazo sensitized, grained aluminum, lithographic printing plate. Another object is to provide a novel coating composition which adheres tenaciously to various supports including metals such as aluminum, zinc, copper, and the like, and to polymeric materials such as polyesters, polyamides, polystyrene, cellulose esters, etc., to provide a hydrophilic coating substantially free from water-soluble materials and to which can be adhered light sensitive coatings, printing inks, paints, etc. Other objects will be apparent from the following disclosure.

The above objects and other objects are attained by making a coating composition in an acid medium of a titanium compound which is substantially water soluble.

A useful source of titanium compound is the titanium orthoesters such as, for example, the tetraalkyl titanates. Although other titanates may be used, the preferred tetraalkyl titanates are those having alkyl groups with 2 to 5 carbon atoms such as, for example, tetraethyl titanate, tetrapropyl titanate, tetraisopropyl titanate, tetrabutyl titanate, tetraisobutyl titanate, tetraamyl titanate, etc.

The acidic constituent which is useful for reacting with the titanate produces a water-soluble titanium complex in an acid media. Useful acidic constituents include, for example, fluosilicic acid, hydrofluoric acid, phosphoric acid, fluoboric acid, etc.

The coating composition is advantageously prepared by adding the alkyl titanate to the dilute aqueous acid,

whereupon the alkyl titanate immediately reacts to form hydrous titanium dioxide which subsequently dissolves and/or reacts forming a hydrophilic titanium complex. When fluosilicic acid is employed to form titanyl silicofluoride, a useful molar range of fluosilicic acid to tetraalkyl titanate is from 5:1 to 1:1 moles, although a preferred molar range is from 2:1 to 1:1 moles. The pH of the coating compositions may be varied from about 1.0 to 5.0.

A useful molar range of fluoboric acid to tetraalkyl titanate is from 7:1 to 2:1 moles.

When phosphoric acid is used as the acidic constituent, hydrogen peroxide should also be used. The resulting complex appears to be titanium peroxy phosphate. The alkyl titanate is added to a dilute hydrogen peroxide solution. When solution is complete, phosphoric acid is then added. In a preferred composition we use 6.8-10.7 moles hydrogen peroxide per mole alkyl titanate and 2.3-7 moles phosphoric acid per mole alkyl titanate. It will be fully realized that the volumetric proportions may be varied and that the amount of water used is not critical but must be sufficient to provide solubility. Hydrogen peroxide can also be used with the other acids.

A useful coating composition is also obtained by preparing a pertitanic acid by dissolving the alkyl titanate in hydrogen peroxide.

Various methods of applying the coating may be used including direct roll, immersion, hopper, knife, wick, bead, spray or any method of convenience. The coating may be on one or both sides of the support.

The thickness of the titanium complex layer on an aluminum substrate is difficult to determine due to its thickness. However, it is most likely in the range of thickness of the naturally occurring oxide.

Drying occurs rapidly, but in production, driers may be used advantageously, employing heat by known means, such as hot air, infrared lamps, etc.

The light sensitive coating may be a suitably stabilized water-soluble resin containing the diazonium group which upon exposure to ultraviolet light forms an oleophilic surface or image.

The light sensitive coating may be of the general formula



where

X' is Cl.

M is a di- or trivalent metal of the groups known to stabilize the diazonium groups, e.g. cadmium, zinc, bismuth, arsenic, antimony, tin, iron, platinum, mercury.

X is an anion or mixture of anions consisting of halogen or sulfates.

Z may be a phenyl or substituted phenyl in which case the resin is an aldehyde condensation product of a p-diazodiphenylamine salt. In this case, Y is hydrogen.

Z and Y may also be organic radicals functionally capable of entering into an addition polymerization, polyesterification, condensation or other reaction capable of producing a relative low molecular weight resin or capable of reacting with a preformed polymer. Z and Y in this case may be the same or different, the parent diazonium compound being a substituted p-diazo aniline.

Some examples of the reactive groups are hydroxyl as in N-ethyl-N-( $\beta$ -hydroxyethyl)-anilino, 4-diazo salts capable of reacting with polymerizable groups such as acryloyl, methacryloyl, etc.

The placement of various groups on the anilino nitrogen can result in the preparation of polyesters, polyethers, polyurethanes, polyacetals, polycarbonates, etc., by direct polymerization or condensation with functionally proper preformed polymers.

In a preferred embodiment, the light sensitive coating consists of an aldehyde condensation product of a p-diazo diphenyl amine. Light sensitive aldehyde condensation products of p-diazo diphenyl amine stabilized with metal salts are well known in the art as described in U.S. Patent 2,714,066. Such resins are also available commercially, e.g. Diazo Resin No. 4, supplied by Fairmount Chemical Co. This material is described as a diazonium sulfate-zinc chloride double salt. However, as stated in the prior art, aluminum reacts with the diazo resin causing decomposition. Therefore, in a preferred embodiment we used a method of preparation and stabilization of the light sensitive diazo resins such that they are less sensitive to decomposition by the aluminum surface.

The presensitized, grained aluminum printing plate prepared according to our specifications, may be handled and treated in use as is customary in the art. The unexposed areas are removed and the plate lacquered, after which the plate is used on a lithographic printing press.

The sensitive layer for the lithographic plate can be exposed to visible light, ultraviolet light, infrared light, X-rays or to heat patterns in order to form differential areas for printing. It is possible to use light sensitive organic compounds such as aliphatic and aromatic esters, hydrazides and amides of naphthoquinone-diazide-sulfonates, cinnamalmalonic acids, their substitution products and functional derivatives, diazonium salts of amino-diphenyl amines and their condensation products with formaldehyde, ortho- and paraquinone diazides of benzenes, anthracenes and heterocyclic systems, for example, quinoline, indazoles, benzimidazoles, diphenyloxides, also diazoketones, unsaturated ketones, ortho- and para-iminoquinone diazides, derivatives of alkylnitronaphthalenesulfonates, nitroaldehydes, acenaphthene, stilbene, azides and diazides and high molecular polymer diazo resins. Silver halide emulsions may also be used. Moreover, the subbing may be overcoated with a photoconductive layer having a high electrical resistance which can be charged and subsequently discharged by light or heat as in electrophotography, for example, low or high molecular weight organic photoconductors, also mixtures thereof with resins. Particularly suitable as photoconductors are oxadiazoles, imidazolones, triazole, oxazole, thiazoles, hydrozones, triazines, polyvinyl carbazole and polyvinyl oxazoles.

Useful resins may contain groups which tend to make the resins soluble in alkali, such groups include acid anhydride, carbonic acid, sulfonic acid, sulfonamide and sulfonimide groups, for example, polyvinyl polymers or mixed vinyl polymers, phthalic acid ester resins, alkyl resins, rosins and polyacrylic acid resins.

The lithographic plates of the invention are further characterized by good adhesion and produce good removal of the unexposed areas so that they can produce a large number of copies.

The drawing shows one embodiment of our invention.

FIG. 1 shows a grained aluminum sheet 3 having thereon a hydrophilic layer produced by treatment with a titanyl salt complex 2 and having thereon a light sensitive stabilized diazo resin 1.

FIG. 2 shows the structure of FIG. 1 following exposure to light and removal of the unexposed areas of the stabilized diazo resin.

The following examples are intended to illustrate our invention but not to limit it in any way.

#### Example 1.—Titanyl silicofluoride

A sheet of brush-grained aluminum having a thickness of 5 mils is immersed in a solution of titanium complex prepared by agitating vigorously a solution of 750 ml. of distilled water in 50 ml. of 31.9% fluosilicic acid, while 10 ml. of tetraisopropyl titanate is added rapidly in a fine stream. The aluminum is then passed between two mechanically driven  $\frac{3}{4}$  inch diameter rubber rolls under sufficient pressure to remove the excess solution. A very thin film of solution is thus obtained which dried rapidly

at room temperature. Similar coatings are obtained on other supports including polymeric material, paper, metal, etc.

Example 2.—Titanyl peroxy phosphate

To 740 ml. of water is added 10 ml. (16.9 g.) of 85 percent phosphoric acid (0.1588 mol) and 30 ml. (33 g.) of 28 percent hydrogen peroxide (0.262 mol). Then with good agitation 10 ml. (9.55 g.) of tetrakisopropyl titanate (0.0336 mol) is added. The result is an orange-yellow solution which is ready for coating. This solution is coated as in Example 1 to give a thin coating on the surface of the support.

Example 3.—Preparation of a titanyl fluoborate coating solution

To 750 ml. of water is added 14.7 g. (0.0672 moles) of 40 percent fluoboric acid with sufficient stirring to mix. To this solution 10.0 ml. (9.55 g., 0.0336 moles) of tetrakisopropyl titanate is added with good agitation. The ortho ester hydrolyzes immediately forming a white precipitate which gradually redissolves forming a clear solution. This solution is then coated on a grained aluminum sheet, dried, and sensitized with a dilute aqueous solution of diazo resin as in Example 5. When properly exposed and processed, as in Example 6, the titanyl fluoborate solution produces a suitable hydrophilic printing surface. Similar coatings are obtained on the supports of Example 1.

Example 4.—Preparation of a pertitanic acid coating composition

Tetrakisopropyl titanate is added to a dilute aqueous solution of hydrogen peroxide in the same manner as the previous example. The white hydrolysis product rapidly turns yellow and gradually dissolves to produce a clear yellow solution. A particularly useful composition for application as in Example 1 contains 0.045 mole per liter of titanium and 0.307 mole per liter of hydrogen peroxide. The hydrophilic character of the surface obtained is enhanced by drying at an elevated temperature. Similar coatings are obtained on the supports of Example 1.

Example 5.—Diazo resin

A diazo resin is prepared by mixing 34 grams p-diazo diphenyl amine sulfate salt with 135 grams concentrated sulfuric acid which has been cooled to a temperature of  $-10^{\circ}$  C. The mixture is agitated while the temperature is maintained at less than  $3^{\circ}$  C. while 3.25 grams paraformaldehyde, and 6.05 grams anhydrous cadmium chloride are added. The viscosity increases over a period of approximately one-half hour and the mixture becomes homogenous. The mixture is then poured over 150 grams of ice and stirred until the ice melts, the yellow precipitate is filtered, redissolved in water and reprecipitated into two liters of isopropyl alcohol, filtered and dried under a vacuum in the dark. Twenty-eight grams are obtained. This resin is a stabilized diazo resin.

Example 6

The treated, grained aluminum of Examples 1 and 2 is then sensitized by immersing in a dilute 2%, aqueous solution of diazo resin, passed between two rubber rolls to remove the excess and dried. When exposed at approximately 24 inches through a negative with a high intensity 220 volt carbon arc in a NuArc Printer, the exposed portions are hardened.

The unexposed portions of the diazo resin are removed by washing with water. The image is then lacquered with a commercially available image lacquer.

The plate is then put on the lithographic printing press and produces 90,000 satisfactory copies. Presensitized plates prepared according to this example are found to have a shelf life for more than two years.

Example 7.—Preparation of a preferred diazo resin sensitizer

An 800 ml. beaker is equipped with a mechanically 75

driven propeller type stirrer and external cooling is provided. To the reaction vessel is added 540 g. (5.35 moles) of 96 percent sulfuric acid followed by portion-wise addition of 138 g. (0.377 mole) of sensitizer DP (para diazo diphenyl amine sulfate, obtained from Fairmount Chemical Co.) with stirring at 25 to  $35^{\circ}$  C. until solution is complete. The mixture is then cooled and maintained at  $0^{\circ}$  C. during the gradual addition of 100 ml. (0.592 mole) of 40 percent fluoboric acid followed by the addition of 13.0 g. (0.432 mole) paraformaldehyde with vigorous agitation to provide rapid and uniform dispersion of the paraformaldehyde. An additional 100 ml. (0.592 mole) 40 percent fluoboric acid is then added. The resultant mixture is now deep red in color whereas prior to the initial addition of fluoboric acid the solution was brownish in color. The reactant mixture is stirred and maintained at  $0^{\circ}$  C. for a period of one hour and ten minutes whereupon it is poured with good agitation into 800 g. ice containing 210 ml. (1.24 moles) of 40% fluoboric acid. The precipitate which forms is then filtered and collected. The moist cake is then dissolved in 700 ml. dimethyl formamide and refiltered. The clear filtrate is then agitated during the addition of 220 g. (0.965 mole) of cadmium chloride ( $\text{CdCl}_2 \cdot 2\frac{1}{2}\text{H}_2\text{O}$ ) dissolved in 250 ml. water. The precipitate thus formed is filtered and collected. The moist cake is then added to 2 liters of isopropyl alcohol and stirred vigorously to produce a small uniform particle size slurry. The slurry is filtered, collected and formed again in the same manner as above in 1 liter of diethyl ether. The slurry is then filtered, collected and dried under vacuum at room temperature, care being taken to break up the moist cake to provide uniform drying. The yield of dry resin is 100 g. in the form of a light orange-yellow powder.

Example 8.—Preparation of a diazo resin sensitizer II

In a 1500 ml. glass beaker was placed 1040 g. of 96 percent sulfuric acid. The beaker was suspended and equipped with a variable speed stirrer. The stirring acid was cooled below  $0^{\circ}$  C. with a Dry Ice-acetone bath.

A 272 g. portion of Fairmount DP salt (Fairmount Chemical Co.) and 26 g. of paraformaldehyde were mixed together thoroughly in the dry state and then added in portions to the acid, keeping the temperature below  $5^{\circ}$  C. The addition took 10 minutes. Stirring was continued for 75 minutes, keeping the temperature below  $0^{\circ}$  C.

The acid solution was poured over a mixture of 2200 g. of crushed ice and a solution of 1 lb. of cadmium chloride in 600 ml. of water with good agitation. A 3 liter portion of isopropyl alcohol was added and the resultant slurry filtered. The precipitate was slurried in 4 liters of water and 3 moles (624 g.) of barium chloride added. The resultant precipitate was filtered off and subsequently extracted twice with three liter portions of 0.75 M HF solution and a third time with 2 liters of distilled water. The filtrates were combined and a solution of 1 lb. of cadmium chloride in 400 ml. added. Then 8 liters of isopropyl alcohol were added and the slurry filtered. The product was dried under vacuum at room temperature. The yield was 286 g.

Example 9

The treated grained aluminum of Examples 1 and 2 is sensitized by coating with light sensitive polymers using the whirler coating technique. Kodak Photo Resist yields a clean appearing image. When inked, 50 press copies are obtained on the lithographic press. Kodak Metal Etch Resist is developed by tray development followed by water wash-off and compressed air dried down to yield a robust, clean appearing image. The image is resistant to prolonged rubbing. Light sensitive compositions of the type described in U.S. Patent 2,948,610 are swab developed with 0.5% sodium carbonate to yield adherent, ink-receptive images. Azoplate Positop developed with Positop

developer yields adherent robust images which show good press life. Light sensitive polycarbonate resins of the type described in U.S. Patent 3,043,802 are tray developed to yield clean, ink-receptive images. A negative working wash-off light sensitive silver halide emulsion is transferred to the treated surface from the strippable support. After activation, the untanned gelatin is washed off.

A light sensitive silver halide emulsion comprising the first gelatin layer containing an oxidizing developer and a second layer containing light sensitive silver halide is coated on the treated support. A satisfactory lithographic plate is obtained after activation and inking of the surface.

The invention has been described in detail with particular reference to preferred embodiments thereof, but it will be understood that variations and modifications can be effected within the spirit and scope of the invention as described hereinabove and as defined in the appended claims.

We claim:

1. A coating composition for providing a hydrophilic layer said composition comprising an aqueous solution having a pH of about 1 to about 5 and containing the complex residues resulting from the dissolution of an alkyl titanate wherein the alkyl group contains 2-5 carbon atoms and at least sufficient solubilizing compound selected from the class consisting of fluosilicic acid, fluoboric acid, hydrogen peroxide, a mixture of hydrogen peroxide and at least one of said acids, and a mixture of hydrogen peroxide and phosphoric acid to maintain aqueous solution.

2. A coating composition as in claim 1 for providing a hydrophilic surface comprising an aqueous solution of a complex of an alkyl titanate and fluosilicic acid in molar ratio from about 1:1 to about 1:5.

5  
10

3. A coating composition as in claim 1 for providing a hydrophilic surface comprising an aqueous solution of a complex of an alkyl titanate and fluoboric acid in molar ratio of about 1:2 to about 1:7.

4. A coating composition as in claim 1 for providing a hydrophilic surface comprising an aqueous solution of a complex of an alkyl titanate and hydrogen peroxide in molar ratio of about 1 to about 6.8-10.7.

5. A coating composition as in claim 1 for providing a hydrophilic surface comprising an aqueous solution of a complex of an alkyl titanate, hydrogen peroxide, and phosphoric acid wherein the molar ratios vary from about 6.8-10.7 moles of hydrogen peroxide and 2.3-7 moles phosphoric acid per mole titanate.

#### References Cited

##### UNITED STATES PATENTS

|           |         |            |       |           |
|-----------|---------|------------|-------|-----------|
| 3,159,613 | 12/1964 | Vandenberg | ----- | 260-91.1  |
| 3,028,297 | 4/1962  | Lagally    | ----- | 106-299   |
| 3,002,854 | 9/1961  | Brill      | ----- | 260-429.5 |
| 2,118,916 | 5/1938  | Drucker    | ----- | 23-202    |

##### OTHER REFERENCES

Chemical Abstract 55: 18,419 F, P. Viallet, 1961 copy in Chemical Library.

JULIUS FROME, Primary Examiner.

THEODORE MORRIS, Assistant Examiner.

30  
25  
30  
U.S. CI. X.R.

96-33; 117-127